

C. D. YOUNG,  
METHOD OF DRYING RAILWAY VEHICLES,  
APPLICATION FILED OCT. 21, 1913.  
1,177,004. Patented Mar. 28, 1916.  
4 SHEETS—SHEET 1.

Fig. 1.



Fig. 2.

Inventor

Witnesses  
Byron B. Collings.  
John Fairbank.

C. D. Young  
T. McWhinney  
Attorney

1,177,004.

C. D. YOUNG.

METHOD OF DRYING RAILWAY VEHICLES.

APPLICATION FILED OCT. 21, 1913.

Patented Mar. 28, 1916.

4 SHEETS—SHEET 2.

Fig. 3.



Inventor

Witnesses  
Byron B. Collings  
G. McFarland

C. D. Young by  
David Thompson

Attorney

1,177,004.

C. D. YOUNG,  
METHOD OF DRYING RAILWAY VEHICLES,  
APPLICATION FILED OCT. 21, 1913.

Patented Mar. 28, 1916.

4 SHEETS—SHEET 3.



### Inventor

Witnesses

Wm. H. Barnes  
Byron B. Collings.  
G. M. Fairbank.

L. W. Young Jr.

F. A. Weihrauch

Attorney

C. D. YOUNG.

## METHOD OF DRYING RAILWAY VEHICLES.

APPLICATION FILED OCT. 21, 1913.

1,177,004.

Patented Mar. 28, 1916.

4 SHEETS—SHEET 4.



Witnesses

Byron B. Collings,  
W. M. Fairbank.

Inventor

C. D. Young

F. G. Weller,  
Special

Attorney

# UNITED STATES PATENT OFFICE.

CHARLES D. YOUNG, OF ALTOONA, PENNSYLVANIA.

## METHOD OF DRYING RAILWAY-VEHICLES.

1,177,004.

Specification of Letters Patent. Patented Mar. 28, 1916.

Application filed October 21, 1913. Serial No. 796,490.

To all whom it may concern:

Be it known that I, CHARLES D. YOUNG, a citizen of the United States, residing at Altoona, in the county of Blair and State 5 of Pennsylvania, have invented certain new and useful Improvements in Methods of Drying Railway-Vehicles; and I do hereby declare the following to be a full, clear, and exact description of the invention, such as 10 will enable others skilled in the art to which it appertains to make and use the same.

This invention relates to a method of drying painted railway vehicles, and has for its object to lessen the time and cost now 15 required to accomplish this end, as well as to improve the life and appearance of the finished covering.

With these and other objects in view, the invention consists in the novel steps, and 20 combination of steps constituting my method, as will be more fully hereinafter disclosed and particularly pointed out in the claims.

Referring to the accompanying drawings 25 forming a part of this specification in which like numerals designate like parts in all the views:—Figure 1, is a diagrammatic cross sectional view in elevation, of an oven suitable for carrying out my invention; Fig. 2, 30 is a perspective detail view of a short pipe section; Fig. 3, is a cross sectional plan view of the parts shown in Fig. 1; Fig. 4, is a longitudinal sectional view of the parts shown in Fig. 1; Fig. 5, is a side elevational 35 view partly broken away of my oven; and Fig. 6, is a longitudinal sectional plan view of the parts shown in Fig. 5.

1 indicates the framework preferably of 40 steel and made to conform to the general shape of a car, 2 any suitable doors for closing the oven during the baking operation, 3 tracks on which a vehicle 4 can be accommodated, 5 an inside lining preferably of steel plate, 6 an outer plate, and 7 45 any suitable lagging between the plates 5 and 6. The doors 2 are insulated in a similar manner.

Along the interior walls of the oven I 50 preferably place a plurality of rows of steam pipe 9, fed from the branch supply pipes 10, joined to the main feed pipe 11 as shown. The pipe 10 may be further provided with extensions 14 joining a plurality of manifolds 12, near the floor, and having tapped 55 into them at intervals the short lengths of pipe 13, as best seen in Figs. 2, 4 and 6.

By this means I am able to provide a very large radiating surface, and with say a steam pressure of one hundred pounds (100 lbs.) I can maintain an oven temperature 60 of 250° F.

Further my structure is such, as will be clear from the drawings, that no metallic connections between the inner and outer surfaces of the oven are had, and therefore 65 the loss of heat from the radiators is reduced to a minimum.

In order to provide for an efficient ventilation the structure has a plurality of preferably rectangular inlets or openings 16 70 near the floor, and a plurality of spaced ventilators 17 of any suitable type in the roof. By this means the fresh air which is necessary for the proper drying of the paint is had, while at the same time an exit is provided 75 for the volatile matter given off. 18 represents suitable drain pipe, and 19 suitable tie members for holding together the frames 1 and stiffening the structure.

In order that my invention may be clearly 80 understood in the case of a car it is said:—A priming coat may be first given the car in the paint shop, whereupon it is moved into the oven and baked for say three hours, the temperature at first being say 160° F. 85 whereupon it may be raised say 1° F. per minute until 250° F. is reached. The oven is now held at this latter temperature for the rest of the three hours, whereupon the car is withdrawn, allowed to cool sufficiently to 90 work upon, and its surfaces glazed and putted where found necessary to fill up depressions and uneven places. The car may now receive its first surfacing coat and be returned to the oven for three hours, baked 95 as before, be removed, cooled and coated again. This may be repeated as often as desired when the outside surface is finally rubbed down with emery cloth and oil and the colors are applied. Each color coat may 100 be baked as above, when the lettering, stripping, etc., is applied, and the varnish coatings are applied. These latter coatings can be likewise baked, but it is preferred to begin the operation at say 120° F. and to not let 105 the temperature rise above say 150° F. The interior of the car is next rubbed to give it a “flat finish” and the painting of the car is completed.

All the above operations can be conveniently carried out with my oven in say from six to eight days, while under the present

system it would require from sixteen to eighteen days to accomplish the same results.

In addition to the above various paints and varnishes have now been prepared so they are especially adapted for this baking process, and are found to have a greater, elasticity, a greater durability, a better appearance and a longer life than those heretofore applied in the old way.

10 It follows from this that the baking process combined with these said paints and varnishes materially lessens the checking and cracking heretofore encountered, and as the work can be done under standard uniform 15 conditions, uniform results are also attained.

Further, I prefer to uniformly heat the car in the first place and thoroughly dry the same before the first priming coat is applied, and by this means all objectionable 20 moisture is removed, and a far better hold is attained by said coat than has been heretofore possible. In other words, before the advent of steel cars, it was not practical to thus heat the wooden cars, and since the 25 advent of said steel cars, no one, so far as I know, has discovered the advantages of making the great surface area of a steel car of a uniform nature so far as moisture is concerned, before applying the priming coat, 30 nor even of making such area uniform for the succeeding coats. This uniformity of surface affording a better grip for my coats, constitutes an important feature of my invention, for it aids in preventing the painted 35 surface from going to pieces in spots as heretofore.

In addition to the above, not only does the coated surface have a longer life, a better appearance, and can be finished in a less 40 time, but the material itself costs less without any extra labor charge.

By the term paint used in this specification I mean the ordinary composition of oil and pigments known as paint, and wish 45 to exclude mixtures of pigments and varnish or mixtures of pigments and Japan or any other like coatings. I greatly prefer to employ my coats of paint without any drying materials at all.

50 It is obvious that those skilled in the art may vary the steps in the process without departing from the spirit of the invention, and therefore I do not wish to be limited to the above disclosure, except as may be required by the claims.

What I claim is:—

1. The method of coating metal car bodies which consists in subjecting the entire body

to a temperature sufficient to drive out the moisture and produce a uniformly dry surface; applying a coat of paint to said surface; and subjecting the entire body and coated surface to a gradually increasing temperature above 160° F. for predetermined periods until a predetermined maximum point is reached and for a predetermined time at said maximum point, substantially as described.

2. The method of coating metal car bodies which consists in producing a uniformly dry 70 surface over the entire body; applying a coat of paint to said body; subjecting said coat to a gradually increasing temperature above 160° F. until the same is uniformly dried; applying a second coat of paint; subjecting 75 said second coat to a gradually increasing temperature above 160° F.; and admitting fresh air to said coats during the drying operations, substantially as described.

3. The process of coating a metal railway 80 vehicle which consists in subjecting the entire body to a temperature sufficient to drive out the moisture; applying a plurality of successive coats of paint of a nature adapted to withstand repeated bakings to said vehicle; uniformly baking each coat by gradually increasing the temperature to a predetermined point; cooling said vehicle and applied coat before each successive coat is applied; suitably finishing one or more coats 90 before applying another coat and admitting fresh air to said vehicle during the drying operations, substantially as described.

4. The process of coating a metal railway vehicle which consists in bringing the vehicle 95 body to a uniform temperature to remove objectionable moisture before applying the priming coat; applying a plurality of successive coats of paint of a nature adapted to withstand repeated bakings to said vehicle; uniformly baking said coats by gradually increasing the temperature, to predetermined degrees above 160° F. for predetermined periods of time; cooling said vehicle and applied coat before each successive coat 105 is applied; suitably finishing one or more coats before applying another coat; and admitting fresh air to said vehicles, substantially as described.

In testimony whereof I affix my signature, 110 in presence of two witnesses.

CHARLES D. YOUNG.

Witnesses:

S. E. GEARHART,  
Otto B. FURRER.